

## UNITED STATES PATENT OFFICE

2,194,518

## BARREL

James Walter Brown, Hammond, Ind., assignor  
to E. I. du Pont de Nemours & Company, Wil-  
mington, Del., a corporation of Delaware

No Drawing. Application January 25, 1937,  
Serial No. 122,117

1 Claim. (Cl. 217—91)

This invention relates to improvements in the manufacture of barrels and is particularly directed to processes for making wooden barrels with iron or steel wire hoops wherein said hoops are rendered resistant to slipping and to rusting by treatment with phosphoric acid.

A wooden barrel is prevented from falling to pieces only by the positions of its parts relative to each other. In assembling a barrel no auxiliary reinforcing means is ordinarily employed, each part, by virtue of its individual location, being relied upon to hold the other parts in their proper places. Movement of any of the parts therefore may cause the barrel to collapse during the assembling operation. It is particularly important that the hoops maintain their proper relative locations.

In the construction of an ordinary wooden barrel the friction between the hoops and the staves is relied upon to hold the hoops in place. The smooth, curving sides of a barrel present a surface upon which it is very difficult for the hoops to secure a satisfactory grip. The hoops tend to slip away from the bulging section of the barrel toward a section of lesser diameter. Slipping of the hoops in this manner constitutes a serious problem in the manufacture of barrels. This difficulty is most frequently encountered when the friction between the hoops and staves is small, as when smooth, new wire hoops are used.

Barrel-makers have heretofore resorted to the practice of deliberately allowing hoops to rust in order to provide a surface better adapted to grip the smooth sides of a barrel. Such practices as sprinkling new hoops with salt water or damp ashes have been employed to accelerate rusting. By such means the friction between the hoops and staves is increased and barrels of greater strength and rigidity are obtained. When rusty hoops are driven into place, as for instance in assembling a barrel on a driving and tressing machine, the difficulties associated with slipping are avoided.

A barrel put together with rusty hoops, of course, presents an unattractive appearance. The hoops continue to rust, particularly if the initial rusting was accelerated by sprinkling with salt or ashes. It is not feasible to paint wire hoops after they have been set in place on the barrel and thus cover over any rusty coating. Hence the unsightly appearance of such rusty hoops has hitherto been unavoidable. Moreover, the practice of using rusty hoops is accompanied by the further disadvantage that rust is rubbed

off of the hoops onto the staves when the barrels are assembled, causing objectionable discoloration. This discoloration of the staves is increased if the hoops are loosened and redriven. These disadvantages resulting from the use of 5 rusty hoops are all considered seriously objectionable by the users of the barrels.

After a barrel has been assembled, the hoops may be held in place by staples or nails. However, nailing or stapling the hoops into place 10 while the barrel is being assembled, as, for instance, while the barrel is in a driving and tressing machine, is neither convenient nor feasible. Momentarily at least, friction between the hoops and staves must be relied upon to hold the hoops 15 in the position to which they have been driven, and slipping at this stage of the manufacture of barrels has heretofore been avoided only by the use of rusty hoops.

I have found that the assembling of barrels 20 having iron or steel wire hoops may be greatly facilitated and the disadvantages and inconveniences of slipping hoops may be avoided by using hoops which have been subjected to the action of phosphoric acid. Treatment with phosphoric 25 acid imparts to the hoops a surface which is ideally adapted to grip the sides of the barrel. Hoops prepared in this manner before placing on a barrel not only retain their proper positions 30 on the barrel, but they also possess the further 35 advantage of being resistant to rusting. When a barrel is assembled following the processes of my invention, therefore, the advantages heretofore attainable only with rusty hoops are secured and at the same time the disadvantages of rusty 40 hoops are avoided.

When driven into place on a barrel, hoops whose surfaces have been treated with phosphoric acid are able to obtain a firm grip on the curving sides of the barrel. Slipping is eliminated. Assembling of the barrel is greatly simplified, especially when the barrel is assembled 45 by machine.

Iron and steel hoops which have been treated with phosphoric acid possess the further advantage that they are resistant to rust. Barrels made with such hoops therefore retain their more attractive appearance even after considerable exposure to air, moisture, and other corrosive influences. Painting of phosphoric acid-treated 50 hoops is, of course, entirely unnecessary.

There is, moreover, no rusty discoloration of the barrel staves at the point of contact with such treated hoops. The hoops may be removed and redriven as often as desired without detri- 55

mentally affecting the appearance of the container.

Because of its improved appearance, a barrel assembled with phosphoric acid-treated hoops 5 according to a process of my invention enjoys a considerable preference over a rusty-hooped barrel, particularly where the barrel is to be seen by the consumer of its contents.

In the following example a particular application 10 of the processes of my invention is shown for the purpose of illustration. It will be understood that the advantages of my invention may be obtained despite considerable variation from the particular conditions described in this example.

The following example shows the application 15 of a process of my invention to the manufacture of slack barrels:

*Example*

20 Several thousand bright basic iron wire hoops were immersed in a 25% solution of orthophosphoric acid at about 20° C. for about one hour. They were then removed and dried. Barrels were 25 then assembled on a tressing and driving machine, using flat steel hoops as rims and the treated iron wire hoops midway between the bulge and either end of each barrel. When once driven into place, the wire hoops remained without slipping. After each barrel was assembled 30 the flat hoops were nailed into place to serve as rims. The finished barrels were strong and rigid and showed no tendency to loosen up when removed from the assembling machine. The appearance of the treated hoops showed no appreciable change from the soft gray coating imparted by the phosphoric acid treatment, even after the barrels had been submitted to an extended period of storage and use.

35 Other slack barrels were made up in a manner similar to that described above except that the bright iron wire hoops were not treated before use. Difficulty was encountered in keeping the hoops in place while the barrels were being assembled because the smooth wire was unable to 40 obtain a satisfactory grip on the staves. When these barrels were subjected to storage and use the bright, untreated hoops started to rust almost immediately and the coating of rust which eventually developed was so heavy that when the 45 hoops were loosened and driven rust was rubbed

into the staves causing objectionable rust marks. The rusty hoops also gave the barrels an unsightly appearance.

5 In assembling any container comprising a plurality of wooden staves held in assembled relation by iron or steel wire hoops, advantages may be derived from the application of a process of my invention. Such containers as kegs and casks, with rounded, bulging sides, may advantageously be assembled using phosphoric acid-treated 10 hoops. A more common application of my invention is, of course, in the manufacture of barrels as shown in the above example.

15 The manner of treating barrel hoops with phosphoric acid according to the processes of my invention is not limited to any particular conditions of time, temperature, and concentration. The conditions used must be such that the hoops are appreciably attacked by the acid. Ordinarily, this attack proceeds more rapidly at elevated temperatures and higher concentrations, but ordinary temperatures and low concentrations may be used if a longer time is allowed. I prefer to use a solution containing from about 10 to 25% 20 of phosphoric acid at temperatures from about 25 to 100° C. The hoops are retained in the acid long enough to be uniformly attacked by the acid over their entire surface.

25 It is not essential to wash the hoops after removing them from the phosphoric acid, since any 30 residual acid will react with the iron or steel to provide an adherent rust-resistant coating of insoluble iron phosphate. Drying of the hoops is likewise not essential. The handling of the treated hoops is facilitated, however, by drying them 35 as shown in the above example.

30 Various expedients may be adopted in treating barrel hoops with phosphoric acid in order to facilitate rapid, economical handling of the hoops. For instance, dirty or greasy hoops may 40 be subjected to an alkaline wash before immersing in the phosphoric acid.

I claim:

45 A barrel comprising a plurality of wooden staves held in assembled relation by phosphoric acid-treated, slip-resistant, ferrous metal hoops 50 having the characteristic etched, roughened, and rust-resistant surface obtained by immersion of a ferrous metal in phosphoric acid.

JAMES WALTER BROWN. 50